

Patented Aug. 23, 1938

2,128,189

# UNITED STATES PATENT OFFICE

2,128,189

## MOTHPROOFING FABRICS

Lindley E. Mills and William W. Allen, Midland, Mich., assignors to The Dow Chemical Company, Midland, Mich., a corporation of Michigan

No Drawing. Application October 16, 1937.  
Serial No. 169,471

5 Claims. (Cl. 21—5)

This invention relates to the protection of fur, hair, feathers, wool, etc. against the attack of moths. It more particularly concerns the moth-proofing of fabrics.

5 Some agents heretofore employed for moth-proofing are capable of attacking or staining the treated material. Other mothproofing agents are highly volatile and impermanent in nature and are soon dissipated by vaporization from the material to which they are applied. Temporary protection has also been afforded by compounds which are soluble in water or soap solutions and in the common petroleum distillate cleaning compositions. Some protecting agents, such as 10 the phenols and mercury and fluorine compounds, are irritating to the skin and poisonous to human beings, while others are objectionable because of their characteristic odor or flammability. A further disadvantage in the use of 15 many of the common mothproofing compositions is the fact that the residues deposited in the treated article following evaporation of liquid constituents are crystalline and are soon dusted out of woolen material and the like.

20 Among the objects of this invention is to provide a method for the protection of the aforementioned materials which will (1) give relatively permanent protection therefor against attack by moths, and (2) yield a protected product free 25 from objectionable odor, flammability, or toxicity to humans. Another object is to provide a composition comprising a volatile organic solvent having dissolved therein a mothproofing material which, upon application to the material, will prevent attack by moths without staining or otherwise injuring the material.

We have discovered that the above advantages can be obtained by employing mono-phenyl-di-(ortho-xenyl)-phosphate as a mothproofing agent. When this compound is incorporated with a suitable organic solvent, and particularly with an alcohol, or liquid halogenated hydrocarbon, and the solution so formed thereafter employed in the mothproofing of woolen fabrics and the like, the articles so treated are not stained or attacked thereby, or caused to develop any distinctive odor, or to become toxic to humans. Furthermore, mono-phenyl-di-(ortho-xenyl)-phosphate is not appreciably removed from the fabric impregnated therewith by the action of water, soap solutions, or common petroleum distillate cleaning fluids, by weathering, or by volatilization or sublimation of the compound, hence retains its effectiveness permanently.

Mono-phenyl-di-(ortho-xenyl)-phosphate is

an odorless water-white liquid boiling at 273°—275° C. at 0.5 millimeter-pressure and having a specific gravity of 1.198 at 60°/4° C. This compound may be dissolved in a solvent carrier in amounts ranging between 1.0 and 7.5 per cent by weight thereof, such solution being advantageously employed as a mothproofing composition. A solution containing between about 3 and about 5 per cent by weight of the agent is satisfactory.

In the numerous tests carried out to establish 10 the efficacy of mono-phenyl-di-(ortho-xenyl)-phosphate as a mothproofing agent, the larvae of the black carpet beetle (*Attagenus piceus*) were employed. This insect is a common household pest, attacking woolens, furs, and other materials. It is particularly destructive to fabrics used in upholstered furniture and to woolen carpets and rugs. It is more resistant and harder to control than the common case-making 15 clothes moth or the tapestry moth, and concentrations of material found suitable for its control on fabrics have been shown to be more than 20 adequate for the control of the latter species.

The following examples are illustrative of certain modes in which our invention may be applied, but are not to be construed as limiting the 25 same.

### Example 1

A number of samples of white wool mohair cloth were saturated with 3 and 5 per cent solutions of mono-phenyl-di-(ortho-xenyl)-phosphate in ethyl alcohol, thereafter pressed to remove excesses of the treating fluid, and allowed to dry. On two of each of these samples 5 larvae of the black carpet beetle were placed and the 35 samples folded over the larvae. These infested cloth samples were placed in a closed cardboard box and examined after periods of one, two, and three weeks to determine the amount of feeding or other attack directly attributable to the beetle 40 larvae. Simultaneous tests were made with larvae upon untreated samples of the mohair, both control and test samples being thereafter incubated at temperatures of 85°—90° F., and at a relative humidity of 70—75 per cent. Examination of the incubated samples impregnated with the 3 and 5 per cent phosphate solutions showed 45 that after three weeks there had been no feeding by the larvae. In each instance one of the 5 larvae was dead on the samples impregnated with 5 per cent phosphate solution. In the case of the untreated controls, there was very slight feeding by the larvae after one week, moderate feeding after two weeks, and heavy feeding at the end of three weeks incubation. Tests carried out 55

## 2

over the same period upon mohair treated by immersion in ethyl alcohol and petroleum distillate alone showed moderate feeding by the larvae after one week, moderate feeding after two weeks, and heavy feeding at the end of the three-week period.

## Example 2

Samples of the impregnated mohair described in the foregoing example were thoroughly dried and then immersed and well washed in an excess of a petroleum distillate dry-cleaning fluid. These samples were dried and exposed to carpet beetle larvae as described in Example 1. Of the mohair samples originally impregnated with the 3 per cent phosphate solution, one sample showed no feeding at the end of two weeks, with very slight feeding at the end of three weeks. The other sample showed no feeding at the end of three weeks. The samples originally impregnated with a 5 per cent phosphate solution showed no feeding at the end of three weeks.

## Example 3

Samples of the woolen mohair fabric, following impregnation as described in Example 1 with 3 and 5 per cent solutions of mono-phenyl-di-(ortho-xenyl)-phosphate, were dried and thereafter weathered out-of-doors for a number of days exposed to sun, wind, and rain. When carpet beetle larvae were introduced into these samples, none of them showed any feeding after three weeks' incubation.

## Example 4

Samples of the impregnated woolen mohair, after drying, were thoroughly washed in a 0.5 per cent solution of Ivory soap in water at a temperature of 40° C. After 20 minutes' contact with the soap solution, these test samples were rinsed in running water and dried. Upon infestation with the carpet beetle larvae, it was found that after two weeks' incubation none of the impregnated samples were attacked, while after three weeks only one of the samples showed a very slight injury which might have been attributable to attack by the larvae.

## Example 5

In a similar manner woolen cloth was impregnated with a 5 per cent solution of mono-phenyl-di-(ortho-xenyl)-phosphate in carbon tetrachloride. Following infestation with the black carpet beetle larvae and incubation for three weeks, the cloth was found to be unattacked by the beetle larvae and to be unaltered as regards physical characteristics.

In the foregoing examples no staining of the impregnated cloth was observed and the fabric itself was not attacked by the phosphate compound. The impregnated cloth in each instance was odorless, and even after prolonged weather-

ing, showed no discoloration. The preservative showed no tendency to crystallize out or to volatilize from the impregnated fabric, nor was the fabric greasy or oily to the touch.

Mono-phenyl-di-(ortho-xenyl)-phosphate has been found to be substantially non-toxic to humans and animals. For example, oral toxicity determinations show that this compound is without effect upon rabbits in the amount of 3 grams of the phosphate per kilogram of body weight of the rabbit. This compound is highly non-flammable and has been found of value for reducing the flammability of textile materials and ligno-cellulosic products generally.

Other solvents for mono-phenyl-di-(ortho-xenyl)-phosphate, forming solutions which may be employed as a mothproofing agent, are liquid halogenated hydrocarbon compounds such as chloroform, ethylene chloride, trichloro-ethylene, chlorobenzene and the like; hydrocarbon compounds such as benzene and toluene; and alcohols such as methyl and isopropyl alcohol; etc. Perfumes, coloring agents and the like may be incorporated in the mothproofing fluid, if desired.

When the mono-phenyl-di-(ortho-xenyl)-phosphate is dissolved in a water immiscible solvent, such composition may be employed as an emulsion with a soap, or other wetting or emulsifying agent, and water. Any of the cleansing agents and detergents common to the cleaning art may then be employed in conjunction therewith.

We claim:

1. A process for mothproofing woolen fabrics and other materials subject to attack by moths which comprises treating such material with mono-phenyl-di-(ortho-xenyl)-phosphate.
2. A process for mothproofing woolen fabrics and other materials subject to attack by moths which comprises treating such materials with a composition comprising mono-phenyl-di-(ortho-xenyl)-phosphate dissolved in an organic solvent.
3. A process for mothproofing woolen fabrics and other materials subject to attack by moths which comprises treating such materials with a composition comprising mono-phenyl-di-(ortho-xenyl)-phosphate dissolved in a lower aliphatic alcohol.
4. A process for mothproofing woolen fabrics and other materials subject to attack by moths which comprises treating such materials with a composition comprising mono-phenyl-di-(ortho-xenyl)-phosphate dissolved in a liquid chlorinated hydrocarbon.
5. A composition consisting of material liable to attack by moths, having incorporated therein mono-phenyl-di-(ortho-xenyl)-phosphate.

LINDLEY E. MILLS.  
WILLIAM W. ALLEN.